

# UNITED STATES PATENT OFFICE.

WILLIS A. GIBBONS, OF NEW YORK, AND HERMAN W. RITTER, OF BROOKLYN, NEW YORK, ASSIGNORS TO AMERICAN RUBBER COMPANY, A CORPORATION OF MASSACHUSETTS.

## PERMEABLE SHEET MATERIAL AND PROCESS OF MAKING SAME.

1,427,754.

Specification of Letters Patent. Patented Aug. 29, 1922.

No Drawing.

Application filed March 31, 1921. Serial No. 457,502.

To all whom it may concern:

Be it known that we, WILLIS A. GIBBONS and HERMAN W. RITTER, both citizens of the United States, residing at New York, county 5 and State of New York, and Brooklyn, county of Kings, and State of New York, respectively, have invented certain new and useful Improvements in Permeable Sheet Materials and Processes of Making Same, of 10 which the following is a full, clear, and exact description.

Artificial or imitation leathers have heretofore been made in three general ways; first by coating a fabric backing with nitro-cellulose composition, second by coating it with a rubber composition, and third, by 15 coating it with a mixture of oxidized or polymerized oil suitably compounded. The pliability and weather resisting character of 20 the rubber type has marked advantages over the others. But the rubber composition as well as the other types mentioned have all been unsuitable for wearing apparel, upholstery and like uses on account of their 25 inability to "breathe" after the fashion of leather. None of the prior imitations permitted the escape of water vapor or air and the dissipation of heat so as to afford relief to a wearer of articles made therefrom.

30 This invention aims to provide a permeable sheet material of plastic composition (preferably but not necessarily of vulcanizable rubber composition) that is pliable and porous or transpiratory and to degree 35 if desired even greater than leather. Applied to a backing, it may have substantially the physical properties of the leather which it is intended to supplant. It also aims to provide such permeable sheet material that 40 does not absorb water in liquid form appreciably, whereas leather will get wet or water-soaked. The invention further aims to provide a commercially practical method 45 for producing the material that is feasible at factories with existing or at least well known equipment, that is economical, that permits production in any desired quantities, that yields a product of uniform quality and any desired porosity, that readily per- 50 mits dressing or desirably forming the surface of the finished sheet in imitation of many varieties of leather, and finally, that is applicable to a variety of plastic compositions.

With the specific details of the invention 55 in mind and without intention to limit its

scope more than is required by the prior art, the invention may be said to consist in the discovery that fluid in general and water in particular may be distributively incorporated in plastic compositions and, after sheeting, but before complete or final set of the plastic mix, may be expelled so as to leave minute pores or openings through the composition which may be permanently retained by the complete setting of the plastic in a 60 pliable sheet form.

The invention has been extensively exploited, and the procedure followed with different compounds will now be detailed.

A compound of the following substances 70 by way of example

|                          |     |
|--------------------------|-----|
| Pale crepe               | 100 |
| Zinc oxide               | 10  |
| Para toluidine           | 4   |
| Sulphur                  | 2   |
| Dibutylxanthicdisulphide | 4   |

may be batched on a mill in the usual manner and there combined with a quantity of solvent naphtha which may be varied considerably but satisfactory results are obtained when by weight it approximates that of the rubber (about 66% being preferred). The solvent naphtha in this case acts as a 80 softening agent rendering the mass pasty but not so soft that it cannot be stripped from the relatively cold mill without sticking. Then 100 parts of finely ground cotton fibers, after being saturated with water, may be added to the softened and pasty batch on the mill, the naphtha softened condition of the batch facilitating incorporation of the wet fibers. In this operation more or less water is squeezed out. The retained water 85 constituting a "blowing" agent incidentally stiffens the batch somewhat and renders it less tacky or sticky which is desirable of course. The mixing in of the wet fibers is continued on the cold mill until a uniform 90 blend is obtained. This completes the first 95 step in the process.

It is to be noted however that the dibutylxanthicdisulphide (also denominated oxy normal butyl thiocarbonic acid disulphide) or its equivalent accelerator owing to its 100 powerful nature is more safely added after the rubber has been softened with solvent naphtha or after the incorporation of water and complete mix of the batch ready for calendering or otherwise sheeting.

The next step is to sheet the mix. This may be conveniently done on a calender whose rolls are preferably in this case at least about or slightly above room temperature depending upon the consistency of the batch. And preferably but not necessarily the mix is calendered onto a fabric backing that has previously been thinly coated by spreading or frictioning with a rubber composition of high quality.

Then desirably but not necessarily the calendered sheet may be embossed and varnished or otherwise dressed with or without a preliminary short cure. Likewise optionally, it may be surfaced by "spreading" in a well known manner with nitrocellulose.

The next step is to expel fluid in the aeroform state and the final step is to set the sheet in its porous condition and serviceably permanent. In the instant case, the curatives being rapid, i. e. requiring only ten to thirty minutes' heat at 200° F. (or a longer time at a lower temperature), these steps are accomplished successively in the curing, at the initial and final stages respectively of the heat treatment. The sheet may be cured either in the condition it comes from the calender or after embossing or dressing its surface. The curing may be effected in a wide variety of ways known to the trade, hanging in heated ovens or chambers similar to those employed in the shoe industry being very satisfactory. The temperature and duration of the cure depend upon the curatives employed and the presence or absence of an accelerator, in the instant case twenty to thirty minutes at a rising temperature to 200° F.

During the first few minutes of the cure in the given case, the softening action of the solvent naphtha increases with the rise in temperature, and the water is converted into vapor and expelled as the temperature increases its pressure. Very largely it is thought the vapor follows the path of least resistance afforded by the fibers whose ends are exposed. To secure uniformity in the physical condition of the product, the sheet should remain sufficiently soft during say the first ten minutes of the cure as to permit a large portion of the water passing off in the form of vapor but the period will vary with the composition. A too powerful curing ingredient or a too high vulcanizing temperature is liable to case-harden the surface by forming a skin of partially cured rubber which of course would prevent the uniform exit of the water vapor and thereby develop blisters and a non-uniform appearance in the product. After vulcanization if desired, the material may be dressed with suitable varnish or the like, if not already so. Finishing before final setting is however deemed preferable, one advantage being that the embossed design then stands out

more distinctly or sharply, and another advantage being that sticking of upholstery stocks for instance is prevented during calendering.

If the product desired is relatively thin, dry fibers may be used instead of wet fibers and air entrapped in their mixture relied upon to yield porosity. In such cases, however, the mix is liable to stick to the calender rolls and great care must be taken in its manipulation. The use of dry fibers on the mill does not now appear to be a desirable course as uniform porosity in the products seems somewhat uncertain.

The mixing of the ingredients in preparation for calendering or sheeting may be accomplished variously.

One modification consists in mixing the color and such curatives as practicable with the rubber on the mill and then mixing in ground rags either simultaneously with or prior to the addition of the solvent naphtha. After the rags have been mixed dry and the naphtha has been combined with the rubber, water may be added either in predetermined amount or in excess, in which latter case it is removed by refining or by expressing in a bag. If powerful curatives or accelerators are used they may be incorporated best after the naphtha or after complete mixing and before calendering. The material may then be refined and calendered as already detailed.

Another way of batching preparatory to sheeting consists in mixing the rubber, colors and such curatives as are practicable on the mill as before and then adding the fibrous material. The fibrous material may be either ground or the grinding effected by the vigorous action of the mill rolls. This batch may now be put into a mixer of any suitable kind, such as the well-known Werner & Pfleiderer type having curved blades revolving in a closed casing, and in the mixer combined with solvent naphtha. When the batch in the mixer has been worked to a smooth and uniform dough a measured quantity of water should be added. Powerful accelerators, if used, should be added after the naphtha or even after the water. The quantity of water will vary with the compound employed and especially the quantity of fibers. But the following may be taken as an example of suitable proportions of the ingredients:

|                          |     |
|--------------------------|-----|
| Pale crepe               | 100 |
| Zinc oxide               | 10  |
| Para toluidine           | 4   |
| Sulphur                  | 3   |
| Ground rag               | 85  |
| Dibutylxanthicdisulphide | 5   |
| Solvent naphtha          | 75  |
| Water                    | 85  |

It has been found that the ground rag

need not be incorporated with the batch on the mill but that it may be worked in in the mixer, which is a further alternative way of making up the batch. After the rubber, 5 minerals, curatives and colors have been batched on the mill they may be removed and put into a mixer together with solvent naphtha and ground fiber. They may then be worked until a substantially uniform 10 dough is obtained. A measured quantity of water—say 75 parts—may then be added, and the mixing continued until it has been uniformly disseminated.

From the foregoing it will therefore be 15 seen that the particular manner of mixing the ingredients so as to incorporate and distribute the fluid and fibers in the plastic may be widely varied. It does not seem to be essential to follow any particular order in 20 adding the ingredients and satisfactory results may be variously obtained, except that in quantity production at the factory powerful curatives and accelerators can be handled or incorporated with less danger after 25 the rubber has been softened with solvent naphtha or after complete mixing and preliminary to sheeting. Vigorous kneading by machines such as mixing mills or mixers would otherwise be likely to cause premature or partial vulcanization.

In the foregoing examples so-called quick curatives were employed these having the desirable property of completely vulcanizing in say ten to thirty minutes at a temperature of 200° F., or less, which is of 35 course commercially advantageous. But the invention is not limited to the use of such quick curatives and is applicable to ordinary vulcanizable rubber compositions.

40 The following:

|                   |                 |
|-------------------|-----------------|
| Pale crepe        | 100             |
| Lamp black        | 20              |
| Litharge          | 30              |
| Solvent naphtha   | 75              |
| 45 Sulphur        | 3 $\frac{1}{2}$ |
| Ground rags (wet) | 85              |

may be employed to produce a porous sheet material. With such materials the procedure is to blend the ingredients on a mill, to then soften with solvent naphtha, and finally to add fibers and water according to the principles already outlined. The mix may be calendered alone or onto fabric and suitably cured in an oven for instance at a temperature of 270° F. for 4 $\frac{1}{2}$  hours.

It has also been discovered that a sheet calendered or otherwise made from a batch of the composition of the first example but 60 without incorporated water may have the pore producing liquid introduced by soaking in warm water for example for about  $\frac{1}{2}$  hour. During the initial stages of its cure or set porosity is developed but not as uniformly as desirable. This method is not

deemed desirable but is comprehended in the broad invention.

It seems therefore that the invention is applicable to vulcanizable rubber compositions generally and that the temperature 70 and duration of cure may be varied widely to suit the composition selected.

Instead of vulcanizable rubber, nitro-cellulose may be employed as the fiber binder. The following:

|                     |           |
|---------------------|-----------|
| Pyroxylin           | 12 grams. |
| Castor oil          | 12 "      |
| Cotton fibers (wet) | 10 "      |
| Amyl acetate        | 200 c. c. |
| Benzol              | 125 c. c. |
| Carbon black        | 1 gram.   |

may be made into a porous imitation leather. The pyroxylin and castor oil may be dissolved in amyl acetate and thinned with benzol to a relatively fluid consistency, and the wet fibers stirred in. The mix may then be spread on fabric with a knife or "spreading" machine and dried between coats at a temperature of approximately 100° C., as 90 many as twenty-five coats being applied if desired.

In this connection it is noted that nitro-cellulose may be blended with a vulcanizable rubber composition and so as to extend 95 throughout the thickness of the sheet, or as an intermediate coat between the plastic base and the finished surface or as a finishing coat on the rubber alone or blended. With upholstery where a surface not frictionally opposing sliding contact is desirable, a cellulosic surface dressing is of advantage.

A permeable sheet material may be produced by incorporating gas. This has been 105 mentioned already in the making of a very thin sheet, it having been found possible to entrap air with dry fibers into the naphtha softened plastic on the mill. But as before intimated, this procedure does not yield uniform results, and is not as reliable as the methods involving the use of a liquid, especially a non-solvent, such as water, to produce porosity or permeability. More 110 satisfactory results with air or gas may be obtained with the plastic or vulcanizable rubber of a fluid like consistency permitting the fibers (either wet or dry, but the former preferably), to be stirred thereinto. The air or gas in this case is entrapped with the 120 fibers during the stirring operation. If desired, the air entrapped with the fibers may be augmented by blowing or otherwise disseminating free air into the mixture. Or the entrapped air may be supplemented by including in the compound light, air-occlusive materials, such as magnesium carbonate, approximating the weight of fibers employed, which latter by weight, preferably 125 approximate the amount of rubber in the ce- 130

ment. The more or less fluid batch obtained may be sheeted as desired with a knife or on a spreading machine having a steam chest in rear of its immersion rolls on which chest the sheet may be passed and dried so as to leave the sheet porous. If vulcanizable, the sheet is then preferably, but not necessarily, subjected to a vulcanizing heat.

The product of all the various methods 10 above outlined is a transpiratory or air-permeable sheet material freely flexible and in most cases having the appearance and feel of leather, and substantially its resistance to abrasive scuffing. It will not absorb water 15 to an objectionable extent and ordinarily hardly to an appreciable extent depending of course upon the diameter of the pores. Its heretofore-unattainable-property of passing air or water vapors renders it practical 20 as a substitute for leather, and therefore adaptable for articles of wearing apparel to a degree not attained by its predecessors. The porosity, transpiration, or air-permeability (however its "breathing" quality may 25 be termed) is believed to be due to the expulsion of aeriform fluid (vapors of the water or mingled vapors of solvent and air or other gas, or of the air or gas alone) prior to the complete setting of the material in a 30 permanent serviceable condition. The expulsion occurs before set or vulcanization has reached the stage of sealing off or case hardening the surface of the sheet. The pores or openings are minute, being scarcely 35 visible, but they impart to the finished sheet the appearance and feel of leather, giving as it were a "grain." By suitable embossing the material may be made in imitation of almost any variety of leather.

40 If the proportion of fibers is varied, the physical appearance of the material may be altered. Insole stock for instance, more nearly resembling felted materials than leather, can be made from

|                               | Parts. |
|-------------------------------|--------|
| Pale crepe                    | 100    |
| Zinc oxide                    | 30     |
| Sulphur                       | 1      |
| Tribenzyltrimethylenetriamine | 3      |
| Dibutylidixanthicdisulphide   | 5      |
| Ground rags                   | 150    |
| Water                         | 75     |
| Solvent naphtha               | 75     |

55 Instead of tribenzyltrimethylenetriamine in the above formula, aniline in the same proportion may be employed as an accelerator, where it has no intolerable effect on the colors employed. The materials may be 60 compounded on a mill or mixer, then sheeted on a calender according to the steps first detailed, and cured in twenty to thirty minutes at a rising temperature to 200° F.

Taking calf-skin as a standard, and as-

suming its transpiration or air permeability 65 is 100, sheet material made by incorporating a gas or air has been obtained with a transpiration substantially as high as leather. With water incorporated to "blow" or produce pores, a transpiration of 200 or even 70 higher may be obtained. Tests for transpiration may be made by placing water in a container with the material covering the mouth and above the surface of the water, the margins being hermetically sealed. The 75 container may then be allowed to stand for twenty-four hours at a temperature of about 20° C. The loss in weight due to the passage of water vapor out through the material to the exterior forms a basis of comparison with leather which had been subjected to the same treatment.

In the basic or broad process the first common step is to mix filler and plastic materials and distributively incorporate fluid 85 therein. The preferred procedure is to mix the ingredients on a mill or in a mixer or both and to incorporate water as the "blowing" agency. Such a course is more practical at the factory, yields a uniform product 90 for any selected composition, and requires the least expense. The batch may be thus prepared in a calenderable condition and calendered in sheet form alone or onto either a permanent or a temporary backing 95 and the procedure is feasible for the manufacture of insole material where there is a large field for its use. Water hitherto regarded intolerable acts with surprising excellence as a pore producing agency. It is 100 cheap, available, and reliable, and permits embossing or dressing the surface of the sheet stock before vulcanization or before complete setting in a wider variety of ways without danger of altering the porosity, 105 which property, in its use, is not developed until the sheet is subjected to heat. Where the incorporated fluid is air, the embossing and dressing is liable to alter the porosity and the final permeability is uncertain. But 110 with water or its equivalent, the surface may be embossed with impunity or dressed with nitro-cellulose or suitable varnish. The vapors of water may be relied upon to produce porosity not only throughout the base 115 composition but also through the surface dressings, the sheet being porous or permeable through and through.

The second general step in the method, to wit, sheeting the mix, comprehends rolling or spreading the plastic (with a calender or a spreading machine), and in the former case at least either alone or onto a fabric backing or onto a temporary backing that is subsequently stripped. Insole stock, for 120 instance, is preferably or rather more cheaply made without a backing. Imitation leathers, on the other hand, desirably have 125

tensile strength approximating if not equaling or surpassing the particular leather to be supplanted and are preferably made by applying the mix to a fabric backing of appropriate strength and texture. And while it is preferred to apply the mix to only one side of the fabric, both sides of the fabric may be coated. Calendering is of course preferred to spreading but the latter has limited fields of usefulness.

The next step, expelling the incorporated blowing agency, may be performed in any suitable manner preferably however in the "spreader" process by passing the sheet onto a steam chest and in the "calendering" process in the first stages of the curing operation. But however effected it is essential to expel or "blow" a substantial portion at least of the incorporated fluid out of the sheet before the plastic sets or hardens. All need not be expelled at this time. Care must be exercised to guard against "case" or "skin" hardening, i. e. surface setting, before the porosity has been adequately developed. The porosity develops in the first few minutes and is usually complete in about ten minutes even when water is used.

When the spreading method is followed expulsion of the incorporated fluid occurs on the steam chest (if used) and necessitates careful manipulation of the sheet in getting it into a heater, if the plastic is vulcanizable. If the plastic is not vulcanizable, the sheet may be completely set on a steam chest or by standing for a sufficient length of time at a suitable temperature, the higher the temperature the shorter time consumed in completely setting the sheet. But very high temperatures over say 250° to 300° F. are dangerous and are to be avoided.

In any case, the expulsion of the incorporated fluid should be effected in the absence of substantial mechanical pressure, i. e. confinement by metal preventing free exit of the incorporated pore producing fluid.

The final step is to set the sheet. If the plastic is vulcanizable this may take place in a room at ordinary temperature or higher, or in a shoe-type of heater, or in open steam, or while the sheet is buried in talc, or in any other suitable manner, depending of course upon the curatives employed and the presence or absence of an accelerator. If the plastic is not vulcanizable the setting may take place at ordinary room temperatures, but preferably at temperatures elevated to suit it. It is also advisable to set the sheet while free of substantial mechanical pressure so as not to alter its porosity, but a mild mechanical pressure not preventing a substantial escape of trapped air or vapor may be used particularly with incorporated liquid such as water where the composition and

thickness of the stock permits and a high 65 porosity is not sought.

The preferred plastic is a vulcanizable rubber composition and quick curing (that is to say, curable in a short time of twenty to thirty minutes, at a temperature of not 70 more than 200° F. and preferably less). But vulcanizable rubber compositions in general, not quick curing, may be employed. In its broadest aspects the invention, however, is not limited to rubber compositions but includes plastics that may be set in a permanently pliable condition. An example of a suitable pyroxylin compound has been given which may be rendered porous after the underlying principle in this invention. 75

Broadly, the invention comprehends the use of any suitable fluid for obtaining porosity. Water, air and gas have been mentioned. But any liquid non-solvent of the plastic and having a high vapor pressure, such as alcohol or aqueous solutions vaporizable at certain different degrees of temperature, may be employed so long as the substance in solution does not deleteriously modify the action of other ingredients in the 80 compound selected. The porosity of the product varies with the composition of the batch both as to proportions, nature and amount of the ingredients particularly of course the plastic binder and fibers. By the 85 methods of manipulation the product is also effected but experience in a short time will enable this factor to be controlled. The easiest way to regulate the degree of porosity is to vary the amount of incorporated 90 pore producing agent and of the various ones mentioned water is the best. 100

Solvent naptha, that is the distillate of coal tar having a boiling point between 300° and 400° F., is the preferred softening agent 105 as it facilitates incorporation of fibers on the mill or in a mixer in the formation of a calenderable mass, and permits mechanical working of quick-curing rubber compounds. but any of the so called solvents or softeners 110 of rubber appear to be equivalents of the solvent naptha in that they soften; the coal tar hydrocarbons such as benzol, toluol, xylol, naphthalene, anthracene, or anthracene oil; and the aliphatic hydrocarbons chiefly petroleum products such as naptha, gasoline or kerosene oil. The softening agent also assists in obtaining porosity. 115

The preferred filler material is cotton fibers, such as may be derived by grinding 120 rags. Not more than 2½ parts of fiber to 1 part of rubber or plastic binder should be used, the less fiber the greater the pliability and tenacity of the sheet. Ordinarily the fibers will be ground before incorporation into the plastic but to a certain extent the mixing operations may be relied upon to reduce the fibers to the proper state of fine- 125

ness. Other fibrous materials that may be satisfactorily used are mechanical wood pulp, chemical wood pulp, newspaper, cotton linters, and hull fibers. Any vegetable 5 or animal fiber is apparently available.

The thickness of the sheet product having the desirable breathing property may be varied widely, porosity having been obtained in the calendering method and using water, 10 in a sheet as much as one-half an inch thick. Ordinarily however, the sheet product will be comparatively thin, if a backing is employed about twice the thickness of the fabric alone, and in the case of insole stock 15 about one-sixteenth of an inch thick. The "blowing" or expulsion of the pore producing agency seems to increase the thickness of the stock.

In the foregoing, it has been endeavored 20 to fully and explicitly disclose the nature of the invention which is believed broadly new. It is to be understood therefore, that the same is not limited to any details not essential to the production of a pliable porous 25 sheet material, and reference should be made to the claims for an understanding of its scope.

In the claims the expressions "permanently pliable" and "permanently porous" 30 have been used to denote properties that are retained by the product during its normal life or service and not everlastingly for all time.

Having thus described our invention, 35 what we claim and desire to protect by Letters Patent is:

1. An artificial pliable and air-permeable sheet material of plastic-bound unwoven and unfelted fibers.

40 2. An artificial pliable and air-permeable sheet material of plastic-bound unwoven and unfelted fibers having substantial resistance to abrasion.

3. An artificial pliable air-permeable imitation leather consisting of unwoven and unfelted fibers bound by plastic and secured to 45 a strain resisting backing.

4. An artificial air-permeable sheet material consisting of unwoven fibrous material 50 bound by vulcanized rubber composition.

5. An artificial pliable and air-permeable sheet material consisting of unwoven fibrous material bound by vulcanized rubber composition and having substantial resistance to 55 abrasive scuffing.

6. An artificial pliable and air-permeable sheet material consisting of unwoven fibrous material bound by vulcanized rubber composition and having substantial resistance to 60 abrasive scuffing and of a leather-like grain.

7. An artificial pliable and air-permeable sheet material consisting of unwoven fibrous material bound by vulcanized rubber composition and having substantial resistance to 65 abrasive scuffing and the appearance and

feel of leather adapted to the same kind of service.

8. An artificial pliable air-permeable imitation leather consisting of fibers bound by vulcanized rubber composition and to a 70 strain-resisting backing.

9. A pliable porous sheet material containing fibers and binding vulcanized rubber composition, the weight of fibers being not more than  $2\frac{1}{2}$  times the weight of rubber in 75 the composition.

10. A pliable porous sheet material consisting of fibers embedded in vulcanized rubber, bound to a fabric backing, and surfaced with nitro cellulose, the whole being air- 80 permeable.

11. An artificial air-permeable and permanently flexible sheeted material of unwoven and unfelted fibers bound together by a plastic and substantially non-absorptive of 85 water.

12. That method of making a permeable sheet material which includes mixing fibrous and plastic materials and distributively incorporating fluid therein, sheeting the mix, 90 gently expelling incorporated fluid with the sheet substantially unconfined by rigid metal members, and finally setting the sheet in a pliable permeable condition.

13. That method of making a permeable 95 sheet material which includes mixing fibrous material and vulcanizable rubber composition and distributively incorporating fluid therein, sheeting the mix, subjecting the sheet to sufficient heat to gently blow aeriform fluid therefrom and leave it porous without confining metal restricting the exit of the fluid, and finally completely vulcanizing the sheet at a temperature suited to its composition.

14. That method of making a permeable sheet material which includes mixing fibrous and plastic materials and distributively incorporating fluid therein, sheeting the mix onto fabric, gently expelling incorporated 110 fluid with the sheet substantially unconfined by rigid metal members, and finally setting the sheet in a pliable permeable condition.

15. That method of making a permeable sheet material which includes making a mix 115 of calenderable consistency of fibrous plastic and a disseminated blowing agency, calendering the mix to form a sheet of the desired thickness, gently expanding and expelling the blowing agency while the sheet is substantially free of confining metal, and finally setting the sheet in a pliable and porous condition.

16. That method of making a permeable sheet material which includes making a mix 125 of calenderable consistency of fibrous material and vulcanizable rubber composition and distributively incorporating a blowing agency therein, calendering the mix to form a sheet of the desired thickness, gently ex- 130

- panding and expelling the blowing agency while the sheet is substantially free of confining metal, and finally setting the sheet in a pliable and porous condition.
- 5 17. That method of making a permeable sheet material which includes mixing filamentary and plastic materials and distributively incorporating a vaporizable liquid therein, sheeting the mix so as to retain disseminated a substantial portion of the liquid, subjecting the sheet to heat sufficient to expel vapors at least of the liquid, and finally setting the sheet permanently pliable and porous.
- 10 18. That method of making a permeable sheet material which includes mixing filamentary material and vulcanizable rubber composition and distributively incorporating a vaporizable liquid therein, sheeting the mix so as to retain disseminated a substantial portion of the liquid, subjecting the sheet to heat sufficient to expel vapors at least of the liquid, and finally setting the sheet permanently pliable and porous.
- 15 19. That method of making a permeable sheet material which includes making a substantially uniform and cohesive mix of fibrous and plastic materials and of a liquid non-solvent of the plastic, sheeting the mix so as to retain disseminated a substantial portion of the liquid, subjecting the sheet to heat sufficient to expel vapors at least of the liquid, and finally setting the sheet permanently pliable and porous.
- 20 20. That method of making a permeable sheet material which includes making a substantially uniform and calenderable mix of fibrous material and vulcanizable rubber composition and of a liquid non-solvent of the rubber, calendering the mix to form a sheet and retaining disseminated a substantial portion of the liquid, subjecting the sheet to heat sufficient to expel vapors at least of the liquid, and finally setting the sheet permanently pliable and porous.
- 25 21. That method of making a permeable sheet material which includes making a substantially uniform and cohesive mix of fibrous and plastic materials and of water, sheeting the mix so as to retain disseminated a substantial portion of the liquid, subjecting the sheet to heat sufficient to expel vapors at least of the water, and finally setting the sheet permanently pliable and porous.
- 30 22. That method of making a permeable sheet material which includes making a substantially uniform and calenderable mix of fibrous material and vulcanizable rubber composition and of water, rolling out a sheet of the mix so as to retain disseminated a substantial portion of the liquid, subjecting the sheet to heat sufficient to expel vapors at least of the water, and finally setting the sheet permanently pliable and porous.
- 35 23. That method of making a permeable sheet material which includes making a calenderable mix of rubber composition, quick curing ingredients, fibers, a softening agent facilitating mixing and calendering, and a liquid non-solvent of rubber, calendering out a sheet of the mix, finishing the surface of the sheet as desired, subjecting the sheet to heat so as to expel vapors of the non-solvent liquid and form minute passages therethrough, and finally vulcanizing the sheet completely.
- 40 24. That method of making a permeable sheet material which includes making a calenderable mix of materials including rubber, quick curing ingredients, fibers, solvent naphtha and water, calendering the mix to form a sheet, subjecting the sheet to heat so as to expel vapors of retained water and form pores therethrough, and finally completely vulcanizing the sheet in a porous, pliable and serviceable condition.
- 45 25. That method of making a permeable sheet material which includes making a calenderable mix of materials including rubber, quick curing material, fibers, solvent naphtha, and water, calendering the mix onto one or more surfaces of a strain resisting flexible sheet, subjecting the sheet to heat so as to expel vapors of the water and form pores therethrough, and finally completely vulcanizing the sheet in a porous, pliable and serviceable condition.
- 50 26. That method of making a pliable transpiratory sheet material which includes making a sheet of fibrous and plastic materials and incorporating a vaporizable liquid therein, expelling vapors of the liquid so as to render the sheet porous, and finally setting the sheet in a pliable porous condition.
- 55 27. That method of making a permeable and pliable sheet material which includes sheeting co-mingling fibers and plastic materials, and setting the sheet in a porous permanently serviceable condition.
- 60 28. That method of making a permeable and pliable sheet material which includes making a porous sheet of fibers and vulcanizable rubber composition, and completely vulcanizing the sheet while porous in a permanently pliable and transpiratory condition.
- 65 29. That method of incorporating fibers in a batch of vulcanizable rubber composition which includes, adding to the vulcanizable rubber composition a softening agent reducing its viscosity, and distributively incorporating fibers in the composition while in a softened condition.

Signed at New York, New York, this 25th day of March, 1921.

WILLIS A. GIBBONS.  
HERMAN W. RITTER.